

## 1

2,814,577

## METHOD OF PRODUCING CORROSION RESISTANT COATINGS OF UNIFORM COLOR AND APPEARANCE ON A SUCCESSION OF ALUMINUM PIECES

Nelson J. Newhard, Jr., Oreland, Pa., assignor to American Chemical Paint Company, Ambler, Pa., a corporation of Delaware

No Drawing. Application May 23, 1956,  
Serial No. 586,646

## 1 Claim. (Cl. 148—6.16)

This invention relates to the art of applying a chemically bonded coating to the surface of aluminum or alloys thereof in which aluminum is the principal ingredient, but before stating the objects of the invention, it is desired to refer briefly to certain coating procedures which are now familiar to those skilled in the art.

It is well known that acidic solutions whose principal and essential coating producing ingredients are fluorides, hexavalent chromium and phosphates and/or arsenates are capable of producing decorative as well as corrosion resistant coatings on aluminum and typical examples of such processes are described in U. S. Patents 2,438,877; 2,471,909; 2,472,864; and 2,678,291. Examination of these patents will show that the solutions used in the coating procedures, in general, have a pH of between 1.6 and 2.2 and that the chemical constituents thereof are present in amounts corresponding to the following: Fluoride 0.6 to 12.5 grams per liter; hexavalent chromium expressed as  $\text{CrO}_3$ , 3 to 60 grams per liter; and phosphate ( $\text{PO}_4$ ) and/or pentavalent arsenate ( $\text{As}_2\text{O}_5$ ), 2 to 285 grams per liter. Furthermore, all of these patents indicate that the fluoride content of the bath must be maintained within a certain ratio to the hexavalent chromium content of the bath.

The solutions used in the methods just referred to are very important commercially and for quite a number of years past there has been a growing demand for aluminum bearing such coatings because of their decorative and protective values. However, during continued use of the solutions or baths employed with such processes, the color imparted to a succession of aluminum articles when processed through the same bath tends to vary. Obviously this is a disadvantage especially where the articles being processed are wall panels or sheets because of the desirability of maintaining the appearance of walls substantially uniform in color as well as in texture and corrosion resistance.

In prior practice it has been customary to maintain certain ratios among the chemical constituents of the solutions used such as the fluoride:chromate ratio, etc., and this practice has been primarily concerned with the maintenance of uniformly corrosion resistant coatings. However, as indicated, such practices have been found to be inadequate insofar as maintenance of uniformity in color is concerned. This inadequacy presents a particularly troublesome problem in the architectural field where substantial uniformity of appearance is important.

With the foregoing in mind, the principal object of the present invention will be better understood and more fully appreciated; and this object is the provision of a method of coating a succession of aluminum pieces in a substantially continuous process involving use of a properly replenished solution by means of which it is possible to maintain on each piece substantial uniformity in appearance and color as well as in corrosion resistance.

As a succession of pieces of aluminum are coated, it is, of course, well known that aluminum as well as alloying

## 2

elements in alloys of aluminum, are dissolved in the bath and I have found that this is largely responsible for the marked change in the appearance and color of the work being processed. Additional experience has now shown that the change in color is due in a very large degree to the manner in which the dissolved metal affects the fluoride content of the bath. Ordinary chemical analysis may show that a used bath has the same total fluoride:chromate ratio as did the original bath but, despite this, the color which it imparts to a coated surface is markedly different from the color produced by the same bath when new or fresh. Furthermore, commercial formulations of the kind in question quite often have, as a source of fluoride, a complex fluoride, for the reasons mentioned in the patents referred to. Certain advantages accrue from the use of such complex fluorides but their presence in the bath further complicates the bath chemistry insofar as the fluoride:chromate ratio is concerned.

The present invention is based upon the discovery that, if the maintenance of a set and definite fluoride:chromate ratio is dispensed with and if, for lack of a better expression what may be termed "active fluoride," is kept substantially constant, regardless of the actual fluoride:chromate ratio, the bath will produce corrosion resistant and decorative coatings of uniform color and appearance on a succession of aluminum surfaces. Naturally, the concentration of hexavalent chromium and phosphate or arsenate should be maintained at conventional concentrations by conventional means.

It should be noted that the term "active fluoride" is used herein to mean the ability of the coating bath to etch a piece of lime soda glass as measured by weight loss.

In order to carry out the present invention all that is necessary is to make up a coating bath in accordance with the knowledge of the art to produce the desired color on aluminum or aluminum alloys and then measure its "fluoride activity." This may be done with ordinary microscope slides of lime soda glass. The measurement is preferably accomplished by heating a convenient volume of the bath to approximately 115° F. and then immersing therein a 4 inch by 3½ inch microscope slide for approximately one-half hour. By taking the weight before and after the immersion, the weight loss is readily determined. As work is processed through the bath, sufficient fluoride is added from time to time as may be necessary to maintain substantially constant the original "fluoride activity."

By way of example, but without limitation as to the specific ingredients or concentrations, work may be processed through a bath consisting principally and essentially of the ingredients given in the following formula:

## Formula

|    |                         |       |    |
|----|-------------------------|-------|----|
| 55 | Sodium bifluoride       | grams | 3  |
|    | Chromic acid            | do    | 12 |
|    | 75% phosphoric acid     | mls   | 35 |
|    | Water, to make 1 liter. |       |    |

60 Such a bath is capable of producing a soft green color when used in a dip process at 100° F. with a treating time of approximately 1½ minutes. In this particular case the "fluoride activity" was measured by immersing a lime soda microscope slide in a part of the bath for ½ hour at a temperature of 115° F. The microscope slide was approximately 4 x 3½ inches in size. The fluoride activity caused a loss of 39.5 mgs. of glass.

To this bath .325 gram of aluminum was added in the form of aluminum phosphate thus simulating the composition of a used bath having the same fluoride:chromate ratio as the bath when new. An aluminum panel was processed with a portion of this bath in a similar fashion

to that given above. The color imparted to the coated panel was of a dull greyish green color and quite different in appearance from the color of the panel coated with a portion of the new bath. The "fluoride activity" of this bath was measured in the same manner as above and found to be down to 17.2 mg. less in weight. An addition of 1.4 grams of sodium bifluoride to the bath brought the fluoride activity back to the level of the original bath. Panels processed in this refurbished bath had the same color as the first panel.

I claim:

In the art of coating a succession of aluminum pieces by subjecting the surface thereof to the action of an aqueous acid coating solution wherein the coating producing ingredients consist essentially of fluoride ions, 15 chromate ions and ions from the class consisting of phosphates and arsenates, the method of replenishing the solution which includes adding thereto compounds contain-

ing chromate ions and ions from the class of phosphates and arsenates sufficient to maintain the required concentrations thereof plus fluoride in sufficient quantity to maintain the fluoride activity of the solution substantially 5 constant as measured by determining the weight loss of a standard piece and type of glass when immersed in the solution for a given period of time at a substantially constant temperature.

10 References Cited in the file of this patent

UNITED STATES PATENTS

2,438,877 Spruance ----- Mar. 30, 1948  
2,679,752 Metler ----- June 1, 1954

15 OTHER REFERENCES

Remy: "Treatise on Inorganic Chem.," page 790, published 1956.

UNITED STATES PATENT OFFICE  
CERTIFICATE OF CORRECTION

Patent No. 2,814,577

November 26, 1957

Nelson J. Newhard, Jr.

It is hereby certified that error appears in the printed specification of the above numbered patent requiring correction and that the said Letters Patent should read as corrected below.

Column 3, line 12, for "coacting" read --coating--.

Signed and sealed this 21st day of January 1958.

(SEAL)

Attest:

KARL H. AXLINE

Attesting Officer

ROBERT C. WATSON  
Commissioner of Patents